

# UNITED STATES PATENT OFFICE.

ALFRED HERZHEIM, OF BERLIN, GERMANY, ASSIGNOR TO THE CHEMISCHE FABRIK AUF ACTIEN, VORMALS E. SCHERING, OF SAME PLACE.

## WATERPROOF PAPER.

### SPECIFICATION forming part of Letters Patent No. 602,558, dated April 19, 1898.

Application filed June 7, 1897. Serial No. 639,729. (No specimens.) Patented in Germany July 27, 1895, No. 86,938; in England November 26, 1895, No. 22,625; in France December 16, 1895, No. 252,501; in Belgium December 16, 1895, No. 118,877; in Hungary June 22, 1896, No. 6,310, and in Austria July 10, 1896, No. 46/2,756.

*To all whom it may concern:*

Be it known that I, ALFRED HERZHEIM, a subject of the German Emperor, residing in the city of Berlin, Germany, have invented 5 new and useful Improvements in Waterproof Paper, (for which I have obtained a patent in Germany, No. 86,938, dated July 27, 1895; in England, No. 22,625, dated November 26, 1895; in France, No. 252,501, dated December 16, 10 1895; in Belgium, No. 118,877, dated December 16, 1895; in Hungary, No. 6,310, dated June 22, 1896, and in Austria, No. 46/2,756, dated July 10, 1896,) of which the following is a specification.

15 This invention relates to the manufacture of water and grease proof paper in a simple and effective manner and without the employment of ingredients which are in any way objectionable with reference to the use of the 20 paper.

In practicing this invention sulfite cellulose is ground or reduced with water in a rag-engine or pulping-machine having dull knives until the cellulose is reduced to a transparent 25 or translucent gelatinous condition, usually from ten to fifteen hours. This mechanical treatment changes the sulfite cellulose to a substance which closely resembles hydrocellulose in its properties. This modified sulfite-cellulose pulp is manufactured into paper in any common and well-known way. 30 This paper is drawn through or immersed in or otherwise coated with a solution of pyroxylin in any suitable solvent—for instance, in 35 acetic ether, a mixture of ether and alcohol,

methyl alcohol, or acetone and alcohol. The solvent of the pyroxylin loosens or softens the surface portions of this kind of paper sufficiently to cause a close and permanent union of the pyroxylin with the paper after 40 the evaporation of the solvent, which union is not destroyed by hot or cold water, weak acids, &c. The evaporated solvent can be recovered by condensation and be again used.

The pyroxylin enters the loosened or soft- 45 ened surface portion of the paper and unites with it so intimately that it becomes permanently united with the paper. The paper prepared in this manner effectually resists the action of warm as well as cold water, grease, oil, 50 and weak acids, and is not easily permeated by air. The paper contains no ingredients which are in any way objectionable in any use to which the paper can be put—for instance, in photography, for packing butter, 55 margarin, grease, substances containing acids, munitions of war, &c.

I claim as my invention—

The herein-described waterproof paper consisting of a body which is composed of the 60 herein-described modified sulfite cellulose resembling hydrocellulose and a coating of pyroxylin permanently united therewith, substantially as set forth.

Witness my hand this 11th day of March, 65 1897.

ALFRED HERZHEIM.

Witnesses:

HENRY HASPER,  
W. HAUPT.